

## UNITED STATES PATENT OFFICE

2,002,180

## CASE HARDENING COMPOSITION

Artemas F. Holden, New Haven, Conn.

No Drawing. Application December 15, 1932,  
Serial No. 647,413

4 Claims. (CL 148—15)

The present invention relates to case hardening compositions which are adapted to become liquid when heated to a proper case hardening temperature and in which the metals to be case hardened are submerged.

The composition comprising my invention is one in which the materials are of such nature that the proper temperature to liquefy the composition and to cause case hardening to occur 10 does not result in fuming when in use, whereby desirable constituents of the composition are not lost as gases.

The articles treated with my composition do not require special washing to prevent rust forming due to the residue of the composition clinging to the case hardened parts. This is particularly important where the case hardened parts are of such form as to present re-entrant angles in which it may be difficult to thoroughly remove 20 the case hardening compound when the case hardening operation is completed.

My composition is such that due to the fact that important parts of the composition are not given off as gases, the bath in which parts are 25 case hardened need only be renewed to make up for mechanical loss of the composition which comprises the amount of the compound which adheres to the parts when they are removed from the bath. In other words, the bath is renewed by 30 adding a mixture of all the constituent parts to the extent of the mechanical loss during the use of the bath. This is an important feature in that the relation of the compounds in the bath does not become unbalanced by the use of the bath.

The composition comprising the present invention is operated at working temperatures beneath 1700° F. and may satisfactorily be used at temperatures as low as 1200° F. Preferably, however, better results are obtained by working between 40 1500° F. and 1650° F., the case hardening depth being more rapid at higher temperatures.

The present composition gives a deeper case hardening depth in a shorter time than has heretofore been attained in any liquid bath. In the 45 use of case hardening compositions, a maximum depth is reached, which depth is not increased by an additional length of time that the parts are treated. The maximum depth heretofore has been approximately one-thirtieth-second of an inch in three hours, and involves the addition at fixed times of definite chemical compounds. The present composition operates more rapidly than the known case hardening compounds and will produce a case hardening which reaches a maximum 50 depth of about one-sixteenth of an inch. In the

use of the present compound with low carbon steel or suitable alloy steels low in carbon content, at a temperature of from 1600° F. to 1650° F. the case hardening depth at the end of one half hour is substantially .008 to .012; at the end of one hour, the depth is .015 to .022; at one and one-half hours, the depth of the case hardening reaches a depth of .025 to .032; and at two hours, the depth is substantially .040 to .045.

In hardness tests, using Rockwell hardness, "C scale", (the "C scale" is one in which a diamond point is used) is substantially as follows:

|                        |          |
|------------------------|----------|
| Half hour              | 55       |
| One hour               | 60       |
| One and one half hours | 62 to 63 |
| Two hours              | 65 to 66 |

The preferred proportions and composition for my case hardening compound are as follows:

|                  | Pounds |
|------------------|--------|
| Sodium cyanide   | 9      |
| Barium chloride  | 6      |
| Barium carbonate | 8      |
| Calcium fluoride | 2 25   |

The above compositions may be varied by equivalents and the proportions may be somewhat varied without departing from the present invention.

The sodium cyanide content should not exceed 30 forty percent of the entire composition and may be as low as fifteen percent of the composition to obtain satisfactory results. The composition may be produced by merely mixing together the above specified constituents or their equivalents without fusing, in which case, the user fuses the composition when the bath is heated. There is a slight fuming at the commencement of the fusing which fuming very quickly disappears. The combined materials may be fused and then 40 broken up as a rough granular structure and transmitted to the user in this form. When so transmitted, the composition remelts at the temperatures specified without fuming.

What I claim is:

1. A case hardening composition adapted to form a case hardening bath for steel articles comprising the fusion of sodium cyanide, barium chloride, barium carbonate, and calcium fluoride and with the sodium cyanide content being between the limits of fifteen percent to forty percent by weight of the total mass.

2. A case hardening composition comprising the fusion of nine parts sodium cyanide, six parts barium chloride, eight parts barium carbonate,

two parts calcium fluoride with parts being designated by weight.

3. A case hardening composition comprising by weight nine parts sodium cyanide, six parts barium chloride, eight parts barium carbonate and two parts calcium fluoride.

4. A fused salt bath for case hardening con-

sisting of a mixture of alkali metal cyanide in an amount sufficient to impart case hardening characteristics to the bath, calcium fluoride, and a barium salt in an amount sufficient to render the bath fluid at relatively low temperatures.

**ARTEMAS F. HOLDEN.**